

April 27, 1943.

J. D. JENKINS

2,317,915

BODYING OF DRYING OILS

Filed April 5, 1940



Inventor

JOHN D. JENKINS

By

Olen E. Bee

Attorney

## UNITED STATES PATENT OFFICE

2,317,915

## BODYING OF DRYING OILS

John D. Jenkins, Forest Hills, Pa., assignor to  
Pittsburgh Plate Glass Company, Allegheny  
County, Pa., a corporation of Pennsylvania

Application April 5, 1940, Serial No. 327,972

7 Claims. (CL 260—407)

The present invention relates to a process of heat-treating drying oils, such as are employed in the formulation of paints and varnishes and the like, and it has particular relation to the process of heat-treating such oils for purposes of increasing viscosity, and improving the rate of drying.

One object of the invention is to provide a drying oil which has a substantially faster drying rate than oils bodied by conventional methods.

A second object of the invention is to provide a process of bodying drying oils which admits of removal and saving of free acids contained in the oil.

A third object of the invention is to provide a process of bodying drying oils by application of which the oil can be easily and quickly bodied to substantially any desired condition with a minimum of apparatus and expense.

A fourth object of the invention is to provide a process of bodying oils which admits of bodying raw oils without "break" formation.

These and other objects of the invention will be apparent from consideration of the following specification and claims.

In the paint and varnish industry, oils of the nature of linseed oil, soy-bean oil, tung oil and the like are employed as film-forming constituents. Before these oils are added to the paint or varnish composition they are often subjected to a process of heat-treatment termed "bodying," which results in a substantial increase in the body or viscosity of the oil and also results in a product which dries more readily than the un-bodied oil. The bodying process has heretofore involved the heating of the oil in a suitable kettle to a temperature of several hundred degrees F. for a period of several hours. Such process is typically a batch operation and necessitates that each batch of oil be carried through a particular cycle of heating and subsequent cooling. The operation is comparatively slow and substantial amounts of apparatus are required in the bodying of the large amounts of oil required in the paint and varnish industry. Periods of heating to bring the oil to bodying and cooling to storage temperature greatly prolong the cycle of operation and make it difficult to judge with accuracy the degree of bodying in the finished product. Operation conditions may also vary somewhat from batch to batch and as a result the uniform-

ity of the product is not always as great as might be desired. Furthermore, the oils contained, or produced during the bodying operation, considerable amounts of free fatty acids which were within themselves valuable for many purposes, such as the formation of artificial resins, plasticizers and other purposes, but under usual operating conditions, were allowed to waste.

Also, by such process it is practically impossible to body raw oils because of separation of a sludge termed "break" where the oil reaches a temperature of about 400 or 500° F.

In accordance with the present invention a drying oil of the type of linseed oil, soy-bean oil, or the like either in the raw or the refined state is subjected to what might be termed a continuous bodying operation, involving the continuous feed of a stream of the oil into a pool of oil of appropriate size in a bodying kettle and simultaneously withdrawing corresponding amounts of the bodied oil. As a further feature the oil in the bodying kettle is continuously blown with an inert gas, such as carbon dioxide or flue gas, or nitrogen in such manner that a proportion of the free fatty acids contained in the oil are blown out and are recovered by condensation or by other suitable treatment.

For a better understanding of the invention reference may now be had to the accompanying drawing in which the single figure is a diagrammatic view of an appropriate embodiment of apparatus suitable for use in the practice of the invention.

In the drawing like numerals refer to like parts throughout. The apparatus may include as a bodying kettle or container 10 formed of any suitable metal. This container is provided with means for supplying heat thereto, for example, it may be partially or completely enclosed or surrounded by the electrical heating coils 11 and a lagging (not shown) for conserving heat. Glyc-  
eride oils, either raw or partially or completely refined are supplied as feed oil to the container 10 through a conduit 12, which as shown in the drawing is so formed at its outlet extremity as to provide a diagonally downwardly-directed lip 13 from which the oil continuously runs as a solid quiescent stream, that flows into the main body of oil in the container 10 with a minimum of splashing or turbulence. The container is, also,

provided with power-driven agitator involving a shaft 14 having propellor blades 16, which are submerged in the oil.

The kettle or container 10 is formed with a slightly conical bottom 17, which at its apex discharges into an outlet conduit 19 having a control valve 21. In order accurately to control the level and therefore the quantity of oil in the container, it may be provided with a constant level overflow pipe, including a vertical portion 22, which may be open at its upper end and at its lower end extends through the bottom 17 to discharge into the conduit 19. The pipe 22 having a valve 25 is provided with a laterally-directed branch 23 disposed at the desired level of the oil in the container and having a downwardly-extending portion 24 opening adjacent to the bottom of the container or kettle in such manner as to insure that the oil flowing off will have been afforded a substantial period of time for heat treatment in the kettle.

As previously stated, substantial amounts of free acids exist in or are liberated in the drying oil as a result of the heat treatment. In order to prevent the ratio of these acids from becoming excessive it is desirable to blanket or to blow the oil with an inert gas, such as carbon dioxide or the like. This is readily accomplished by conducting the gas through a conduit 26 and discharging it adjacent to the bottom of the container. The inert gases escaping upwardly through the oil are discharged through a drum 27 at the top of the container and passing outwardly through conduit 28 to a condenser apparatus comprising a shell 29 of conventional design, involving drum sections 31 and 32 at the top and bottom thereof respectively, and intermediate or connecting tubes 33 through which the vapors and the condensed oil flow downwardly.

The tubes may be cooled by any desired medium, but preferably the inert gas for the blowing operation is used as a cooling medium and is thereby preheated before introduction into the kettle. For this purpose the conduit 26 is connected at its upper end 36 to the shell 29 below drum section 31 and receives gas which is introduced by conduit 34 having an inlet to shell 29 above drum 32 and which is heated in its passage upwardly about tubes 33.

The cooled carbon dioxide from the drum 32 is discharged through outlet conduit 38 and may be dried and otherwise treated preparatory to recycling to the apparatus. It may also be discharged to the atmosphere or employed for other purposes, if so desired. The free fatty acids condensed from the carbon dioxide in the tubes 33 are collected in the drum 32 and are discharged to storage through the conduit 39.

Apparatus for cooling the bodied oil discharge from the container 10 and for preheating the oil for inlet to the container through conduit 12 is indicated at 41. This apparatus includes a water cooler 42 and a heat exchange unit 43 interconnected at their tops by a conduit 44, which in turn is connected to the outlet conduit 19 for the bodied oil. Valves 46 and 47 upon opposite sides of the conduit 19 admit of selectively flowing the hot but bodied oil either to the cooler 42 or heat exchanger 43 or admits of dividing the flow of oil to the two units in any desired manner. The cooler and the heat exchange unit are of substantially identical construction and include shells 48 having upper drums 49 and lower drums 51, which are interconnected by tubes 52 in con-

ventional manner. The space about the tubes in the cooler 42 is filled with cooling medium, such as water, fed thereto through the conduit 53 and discharged at the top of the unit through conduit 54.

The heat exchanger 43 is employed to preheat the feed oil to appropriate temperature, e. g. about 400 to 500° F., which is accomplished by feeding the oil through conduit 59 to the lower portion of the space about the tubes 52, and drawing it off at the top of the same space through outlet 57, which constitutes a continuation of the feed conduit 12. The cooled or partially cooled oil is received in the drums 51 and is discharged into the outlet conduit 61, which interconnects the drums. Conduits 62 and 63, connected to the conduits 61, lead to a conduit 64 through which the bodied oil is discharged to storage.

It is to be noted that by-pass conduits 66 and 67 are connected to conduit 61 intermediate of the unions or connections to the conduits 62 and 63. These by-pass conduits at their upper extremities are joined to the conduit 44 upon opposite sides of the valves 46 and 47. Valves 68 and 69 are provided in the by-pass conduits and also valves 71 and 72 are disposed in the conduit 61 respectively between the by-pass conduits, the cooler 42 and the heat exchanger 43. A valve 73 is further disposed in conduit 61 between the two by-pass conduits. Finally valves 74 and 75 are disposed in the conduits 62 and 63. It will be apparent that by appropriate manipulation of these various valves it is possible to discharge the whole of the bodied oil either into the heat exchanger or the cooler, or the oil may be divided in any desired manner. Furthermore, the oil may be discharged from the heat exchanger and then passed through the cooler or vice versa, depending upon operating conditions which it is desired to obtain. It will be apparent also that, if desired, the oil may be by-passed through conduits 66 and 67 without passing through either the heat exchanger or the cooler.

In the operation of the apparatus as herein disclosed the container or kettle 10 is filled to the desired level with oil with the discharge valve 21 closed. The flow of inert gas and the agitator are started and the oil is then heated to the bodying temperature after which the continuous flow of oil through the conduit 12 is started. The rate of flow, of course, is so adjusted that the oil is allowed to stay in the bodying kettle for the requisite length of time to obtain a satisfactory degree of bodying. This will depend upon the temperature of the kettle and the nature of the oil itself. However, in general the temperature probably will be around 600° F. The average time in the kettle will vary with the degree of bodying required and probably will be of the order of 1 to 10 hours. Oil introduced into the pool in kettle 10 is brought substantially instantaneously to bodying temperature.

The oil may be drawn off, as it is bodyed, through the discharge conduit 19 by merely opening the valve 21 to the requisite degree, or if preferred the valve 21 may be closed and the oil allowed to discharge at the desired rate through the overflow pipe 22. The bodied oil passes off through conduit 19 to the water cooler 42 or the heat exchanger 43 where it is cooled to the desired degree before passing to storage.

The feed of carbon dioxide or other inert gas into the kettle will depend upon the acidity desired in the final product. A certain degree of

acidity is perhaps desirable and may be obtained by increasing or decreasing the flow of inert gas, in order to blow away any excesses of the acids.

The following represent typical operating conditions for the bodying of linseed oil.

TABLE I.—*Lightly bodied linseed oils*

| Feed oil                                  | Refined | Raw      |
|-------------------------------------------|---------|----------|
| Temperature of operation, ° F.            | 603     | 608      |
| Feed rate, gal./hr.                       | 10      | 10       |
| Ave. treatment time, hrs.                 | 2       | 2        |
| CO <sub>2</sub> wt. percent of feed oil   | 9.7     | 6        |
| F. A. distillate, percent of feed oil     | 1.3     |          |
| Ratio wt. CO <sub>2</sub> /wt. distillate | 7.5     |          |
| <i>Properties of products</i>             |         |          |
| Vis., $\frac{1}{4}$ " cup at 25° C., sec. | 11      | 8        |
| Color, Gardner                            | 2.5     | Greenish |
| Acid number                               | 6.7     | 8.35     |
| Iodine value                              | 134     | 136      |
| Refractive index                          | 1.4859  | 1.4852   |
| Crit. sol. temp. (Note 1)                 | 4.0     | Below 0  |
| Drying time, hrs. (Note 2):               |         |          |
| .3% Pb, .03% Mn                           | 5.7     | 6.7      |
| .06% Co                                   | 3.8     | 4.6      |

TABLE II.—*Heavily bodied linseed oils*

| Feed oil                                  | Refined | Raw    |
|-------------------------------------------|---------|--------|
| Temp. of operation, ° F.                  | 608     | 608    |
| Feed rate, gal./hr.                       | 2.5     | 2.75   |
| Ave. treatment time, hrs.                 | 8       | 7.3    |
| CO <sub>2</sub> wt. percent of feed oil   | 38      | 33     |
| F. A. distillate, percent of feed oil     | 8       | 10     |
| Ratio CO <sub>2</sub> /distillate         | 4.8     | 3.3    |
| <i>Properties of products</i>             |         |        |
| Vis., $\frac{1}{4}$ " cup at 25° C., sec. | 210     | 195    |
| Color, Gardner                            | 4       | 5      |
| Acid number                               | 12.7    | 13.9   |
| Iodine value                              | 116     | 115    |
| Refractive index                          | 1.4927  | 1.4924 |
| Crit. sol. temp., 0° C. (Note 1)          | 39.6    | 37.7   |
| Drying time, hrs. (Note 2):               |         |        |
| .3% Pb, .03% Mn                           | 4.8     | 5.3    |
| .06% Co                                   | 2.9     | 2.9    |

Note 1.—50% by weight in acetone.

Note 2.—68° F., 65% relative humidity.

Samples aged 20 hours before testing.

The oils marked in the table as "Refined" were subjected to alkali refinement prior to the bodying operation. The oils marked "Raw" were typical linseed oils without the alkali refinement treatment. The properties of these bodied oils may be compared with those of a typical alkali refined oil which was bodied by a conventional batch process. These properties are tabulated as follows:

TABLE III.—*Batch bodied refined oil*

|                                           |             |
|-------------------------------------------|-------------|
| Vis., $\frac{1}{4}$ " cup at 25° C., sec. | 7-12        |
| Color, Gardner                            | 3           |
| Acid number                               | 4.7         |
| Iodine value                              | 132         |
| Refractive index                          | 1.4837      |
| Crit. sol. temp.                          | Below 0° C. |
| Dry time, hrs.:                           |             |
| .3% Pb, .03% Mn                           | 9.4         |
| .06% Co                                   | 5.0         |

It is to be observed that the alkali refined oil, when continuously bodied by the process herein disclosed, possesses a substantially more rapid rate of drying than the corresponding oil bodied by conventional methods. For example, it will be observed that in the case of the conventional product the drying rates were respectively 9.4 and 5 hours dependent upon the drier which was added thereto. In contradistinction, the alkali refined oil, when bodied by the present process,

dried in periods of 5.7, 3.8, 4.8 and 2.9 hours, dependent upon the catalyst and the degree of bodying. The raw oil dried in periods of 6.7, 4.6, 5.3 and 2.9 hours, likewise dependent upon the catalyst and the degree of bodying to which it was subjected.

The oil when continuously bodied in accordance with the present invention is subjected to substantially different conditions than exist in a conventional batch process. In a batch operation the oil is relatively slowly brought to bodying conditions and all of the oil is subjected simultaneously to the same conditions and there is a tendency for all portions of it to go through the same reactions. The reactions of course include various polymerizations in which monomeric glycerides are added together to form dimers and subsequently dimers are added together or monomer is added onto a dimer and so on.

On the other hand it is probable where the oil is continuously bodied, when the apparatus has been operating for a sufficient period of time for equilibrium to be reached, a very high percentage of the oil in the polymerization zone is in the condition of a relatively high polymer. The feed oil, which at any particular time is present in the reaction mass in only a relatively small amount, is afforded an especially good opportunity for contact and reaction or addition to the higher polymers and there is but little opportunity for contact of monomer with monomer. Therefore, it is to be expected that relatively small amounts of the dimer will be present in the bodied oil and proportionally there will be a relatively large amount of highly polymerized material present. This perhaps tends to explain the relatively high rate of drying of applicant's product.

Applicant's process is of particular value in the bodying of raw or unrefined drying oils, such as linseed, soya bean, and the like, because raw oils, when heated to a temperature of about 400 or 500° F. undergo "break" formation. A slime is produced that for most practical purposes can not be removed. However, in applicant's process, if oil below "break" temperature is run into the pool of bodying oil, the temperature of "break" formation is passed almost instantly and "break" does not separate. The hot oil can then be bodied. A slightly bodied raw oil can be taken off from the apparatus and then batch bodied, if so desired.

The sudden heating seems to result in fixation of the "break" in the oil so that it does not separate during bodying. Presumably the bodied raw oil still contains the break-forming constituents.

It is to be understood that the intermittent or pulsating feed of raw or refined oil into the bodying kettle and corresponding withdrawals of bodied oil is contemplated. Likewise, it may sometimes be desirable to run oil, raw or refined, into a kettle which initially contains only a small amount of oil; however, the latter being at bodying temperature. The addition is so made that the kettle is gradually filled but always the bodying temperature is maintained. When the kettle is full and the oil is sufficiently bodied, discharge is effected.

The forms of the invention herein disclosed and described are to be understood merely as exemplary and it will be apparent that numerous modifications may be made therein without departure from the spirit of the invention or the scope of the appended claims.

What I claim is:

1. A process of bodying without "break" formation raw drying oils from a class consisting of linseed and soy-bean oil, but containing "break-form" constituents, which process comprises continuously feeding unbodied raw drying oil into a pool of oil heated to the bodying temperature, substantially instantaneously admixing the feed oil with the oil of the pool and correspondingly withdrawing the bodied oil, the rate of feed and withdrawal of the oil being so adjusted that the desired degree of bodying is obtained while the oil is in the heated pool, and bubbling into the oil in the pool an inert gaseous medium, in order to remove free acids therefrom.

2. A process of bodying without "break" formation raw drying oils from a class consisting of linseed and soy-bean oil, which comprises bringing the oil from a temperature below that of "break" formation to bodying temperature substantially instantaneously and then maintaining the oil at bodying temperature until a desired degree of bodying has been reached.

3. A process of bodying without "break" formation raw, drying, glyceride oils from a class consisting of linseed and soy-bean oil and containing "break-forming" constituents, which process comprises feeding the oil as a stream into a pool of oil heated to bodying temperature whereby to bring the feed oil substantially instantaneously to bodying temperature, and drawing off bodied oil as raw oil is fed in.

4. A process of bodying without "break" formation raw drying oils from a class consisting of linseed and soy-bean oil and containing "break-forming" constituents, which process comprises feeding the oil at a temperature below that of break formation, as a stream into a pool of oil heated to the bodying temperature and quickly mixing the inflowing oil with the oil in the pool,

5. whereby to heat the feed oil substantially instantaneously to the bodying temperature, and correspondingly drawing off oil from the pool, the pool being of such size that the oil is incompletely bodied while it is therein, and subsequently completing the bodying operation by further heating the oil in a batch operation.

10 5. A process of bodying without "break" formation drying oil from a class consisting of linseed and soy-bean oil and containing "break-forming" constituents, which process comprises running unbodied oil as a free falling stream into a pool of the oil heated to the bodying temperature, the temperature being maintained during the 15 addition, then drawing off the oil after it has been bodied.

6. A process of bodying without "break" formation raw drying oils from a class consisting of linseed and soy-bean oil, but containing "break-forming" constituents, which process comprises 20 flowing the feed oil as a continuous stream into an agitated pool of oil at an elevated temperature under such conditions that the oil becomes substantially instantaneously heated to the temperature of the pool, said temperature being sufficiently high to obviate "break-forming" tendencies in the oil, then subsequently bodying the oil.

25 7. A process of bodying a refined, drying, glyceride oil from a class consisting of linseed and soy-bean oil to obtain a product of drying properties superior to those of the same oil when batch bodied, which process comprises feeding the oil as a stream into a pool of the oil heated to the bodying temperature and substantially 30 instantaneously mixing the feed oil with the heated oil in the pool, maintaining the oil in the pool until it is substantially bodied, and withdrawing bodied oil at approximately the rate at 35 which it is fed in.

40

JOHN D. JENKINS.